

May 16, 1944.

M. FARR, JR

2,349,083

ELECTROLYTIC PROCESS FOR COATING ALUMINUM AND ALUMINUM ALLOYS

Filed May 13, 1940



Inventor

*Michael Farr Jr.*

By

*W. S. Howell*

Attorney

Patented May 16, 1944

2,349,083

# UNITED STATES PATENT OFFICE

2,349,083

## ELECTROLYTIC PROCESS FOR COATING ALUMINUM AND ALUMINUM ALLOYS

Michael Farr, Jr., Columbus, Ohio, assignor to  
The B. & T. Floor Company, Columbus, Ohio,  
a corporation of Ohio

Application May 13, 1940, Serial No. 334,763

4 Claims. (Cl. 204—58)

This invention relates to a process whereby aluminum and aluminum alloys are anodically provided with an even, hard, corrosive-resisting oxide coating.

It is the object of this invention to provide an economical and efficient method for effecting the formation on the outer surfaces of an aluminum or aluminum alloy body of a hard, fine grained oxide coating which, at first, is permeable and adsorbent, adaptable for impregnation with an oil or dye and for subsequent buffing, or may be left in its natural color and buffed. After being buffed, however, the electrolytically formed coating becomes substantially impermeable and non-adsorbent, and when in this latter condition, said coating possessing its maximum hardness. In previous processes of an analogous nature, a comparatively highly concentrated electrolyte and/or a comparatively high voltage are required to produce a coating conforming substantially in quality to that produced by means of my process.

My invention, therefore, consists in the provision of a method wherein the aluminum or aluminum alloy to be treated is made the anode in an electrolyte of about 10%  $H_2SO_4$ , either C. P. or a commercial grade producing satisfactory results. Then a direct current of from six to twelve volts is applied. In this 10%  $H_2SO_4$  electrolyte, using the voltages stated, the amperage is automatically controlled, a feature not considered possible in prior art processes of which I am aware.

As an important feature of my invention, I make use of a special system of electrolysis tanks, which system contributes to the automatic controlling of current flow. In this system, I employ an outer tank, preferably of lead, and which is used as the cathode. Within this outer tank, I position a smaller and inner tank of glass, hard rubber or other suitable non-conductor. The inner tank is supported upon several lead blocks in a manner so that the cellular tank does not actually lessen the effective cathode surface. The inner tank is not quite as deep as the outer tank, so that when the latter is filled to a predetermined level with the electrolyte, the inner tank is completely immersed. By this arrangement of tanks, the resistance of the electrolytic cell created thereby is increased, resulting in a reduced current demand. With this combination of low voltage and low electrolyte density, approximately 1.05 sp. gr., the length of time required to produce a good oxide coating is approximately thirty minutes, longer or shorter immersions producing, respectively, thicker or thinner oxide coatings.

The temperature of the electrolytic bath should not be allowed substantially to exceed 30° C.

In carrying out the process, the total body to be coated is first cleansed of grease, dirt or foreign impurities, in any efficient way. A practicable method is to clean the metal by subjecting the same to a bath composed of a hot solution of lye, although other cleansing agents or solvents may be used. The metal is then rinsed and suitably supported within the confines of the inner tank, surrounded of course by the electrolyte. The lead walls or lining of the outer tank are formed to constitute the cathode of the cell and the aluminum or aluminum alloy to be treated is connected with the source of electrical energy to form the anode. An electric current of from six to twelve volts is turned on for about thirty minutes, the period of such electrolytic activity being varied to meet the demands of the coating thickness. The metal is then removed from the cell, rinsed and dried. At this stage of procedure, the applied oxide coating is relatively porous and adsorbent, possessing a light color. It may now be buffed to impart a desired lustrous appearance thereto, and after such buffing, the coating becomes impervious and non-adsorbent, but retaining its light color. Again immediately following removal from the electrolytic cell, the coating may be impregnated with an oil or a suitable pigment and later buffed, so that various color effects may be obtained.

In the accompanying sheet of drawing, the single figure is a diagrammatic view in vertical section, disclosing my improved tank arrangement. In the drawing, the numeral 1 designates the outer tank, the same being of any desired dimensions, possessing a substantially box-like form with an open top. The inner walls of the tank are preferably provided with a lead lining, as indicated at 2, which lining is used as a cathode of the cell. Positioned upon spaced lead blocks 3, arranged on the bottom of the tank 1 and within the same, is the inner tank 4, this tank being formed from glass, hard rubber or other suitable dielectric which is not affected by the electrolyte 5. As stated, this electrolyte comprises a dilute solution of sulphuric acid of the order above specified.

Supported within the inner tank 4 by wires 6, or other suitable current conveying members, is the article 7 to be treated. In the present instance, a piece of molding has been illustrated, this molding being formed of an extruded aluminum alloy. The supporting wires 6 extend upwardly and are hooked or otherwise connected to a bar 8 to which current is conducted from a

current source of desired potential by a lead 8. The negative terminal of the current source is connected by a second lead 10 with the lead lining 2 to complete the circuit and when current flow is established by the closing of a suitable switch, not shown, an electrolytic action is initiated by which the article 1 will be coated.

It will be noted that the inner tank, which has the same box-like form of the outer tank, has the upper edges of its side walls terminated just below the level of the electrolyte, so that current flow passing through the cell is elongated and compelled to travel through the restricted portions of the bath disposed above the upper edges of the inner tank. This arrangement provides for the automatic controlling of the current flow and distribution thereof in traversing the cell, increasing the resistance of the latter and providing for the coating of the aluminum or aluminum alloy bodies with oxide particles, which under microscopic examination, are exceedingly fine and closely compacted. These features collectively produce a coated aluminum body, wherein the coating is unusually even, hard and resistant to abrasive forces. Moreover, the coating does not smudge upon being handled or when in use nor lose its highly lustrous appearance.

What is claimed is:

1. A process of producing on aluminum surfaces an electrolytic coating which comprises: making the aluminum to be coated an anode in an electrolyte containing about 10% by weight of sulphuric acid, surrounding the aluminum anode with an inner tank composed of a dielectric with said tank completely immersed in said electrolyte, supporting said inner tank within an outer tank comprising an electrical conductor in which the electrolyte is contained at a level above that of the inner tank, said outer tank forming the cathode connection of the electrolytic cell, applying to the electrolytic cell an electric current having a voltage of from six to twelve volts, maintaining the electrolyte at a

temperature not in excess of 30° C., and continuing the application of said current for a period of approximately thirty minutes, said inner tank being located between the anode and

5 the outer tank.

2. In electro-coating articles of aluminum and aluminum alloys, the process of making such an article an anode in sulphuric acid diluted to about 10% H<sub>2</sub>SO<sub>4</sub>, containing the sulphuric acid 10 electrolyte within an outer receptacle forming a cathode, shielding the article to be coated by surrounding the same with an inner tank element composed of a dielectric and completely immersed in said electrolyte, the inner tank element 15 being located between the anode and the cathode, and impressing a current having a voltage of from six to twelve volts on said electrolyte.

3. In electro-coating articles of aluminum and aluminum alloys, the process of making such an article an anode in sulphuric acid, containing the sulphuric acid electrolyte within an outer receptacle forming a cathode, shielding the article to be coated by surrounding the same 20 with an inner tank element composed of a dielectric and completely immersed in said electrolyte, said inner tank element being located between the anode and the cathode, and impressing a current of from six to twelve volts on 25 said electrolyte.

4. A method of electro-coating articles formed of aluminum and aluminum alloys comprising passing an electric current through an electrolyte in which the article is immersed as an 30 electrode to form an anodic film on the surface of the article, surrounding the article while in 35 said electrolyte with a dielectric shield disposed between the article and the cathode, the shield being completely immersed in said electrolyte and being maintained at a constant value between all parts of the article and the cathode, and impressing a current of six to twelve volts on 40 said electrolyte.

MICHAEL FARR, JR.